

## UNITED STATES PATENT OFFICE

2,330,587

## FLOTATION REAGENT AND PROCESS

David Walker Jayne, Jr., Old Greenwich, Conn.,  
assignor to American Cyanamid Company, New  
York, N. Y., a corporation of Maine

No Drawing. Application November 6, 1940,  
Serial No. 364,495

14 Claims. (Cl. 209—166)

This invention is directed to a composition for and a method of froth flotation of ores.

More particularly the present invention relates to a new combination of flotation promoters whereby increased effectiveness is obtained in froth flotation operations.

It has been known in the past that certain diaryl thioureas were promoters in the froth flotation of various ores, as for example lead sulfide ores. Only one of these diaryl thioureas, namely, di-phenyl thiourea (thiocarbanilide) was considered to be sufficiently effective in froth flotation operations to economically justify its use. While it was known that higher homologues of di-phenyl thiourea, such as di-tolyl thioureas and di-xylyl thiourea, had some promoter action, they are very insoluble in water and their action is extremely weak as compared with thiocarbanilide; and as a result, they have not been used extensively in flotation operations. It has also been known in the past that the effectiveness of thiocarbanilide as a promoter could be increased by using a mixture of thiocarbanilide and an organic dithiophosphoric acid, and such a composition is disclosed and claimed in the U. S. Patent No. 2,043,192. Since the promoter action of the higher homologues of thiocarbanilide is much weaker than thiocarbanilide, one would expect that solutions of the higher homologues in organic dithiophosphoric acid would also be weaker.

In accordance with the present invention, it has been discovered that di-tolyl thiourea and di-xylyl thiourea are more effective promoters when mixed with an organic dithiophosphoric acid than mixtures of thiocarbanilide and organic dithiophosphoric acids, in spite of the fact that they are not effective promoters as compared to thiocarbanilide when used alone. This is a result which could not have been predicted in view of the teachings of the prior art. It might have been expected that mixtures of di-tolyl thiourea or di-xylyl thiourea and organic dithiophosphoric acids would be a more effective promoter than di-xylyl thiourea or di-tolyl thiourea alone, but it is obvious that such a combination would be more effective than similar thiocarbanilide combinations.

It is an advantage of the present invention that a class of reagents which were heretofore not suitable as promoters in froth floatation operations are provided in a form which makes them seem

entirely satisfactory as promoters. It is also an advantage that although di-tolyl thiourea and di-xylyl thiourea are practically insoluble in water they are soluble to the extent of about 10% or more in most organic dithiophosphoric acids, whereas the di-phenyl thiourea of the prior art is soluble only to the extent of about 6%. Thus the present invention not only provides a reagent combination which is more effective when used in equal quantities as compared to thiocarbanilide, but also permits the preparation and use of a more concentrated solution. It is a further advantage of the present invention that although many dithiophosphates are promoters, the effectiveness thereof is very materially increased by the addition thereto in solution of even a relatively small amount of either di-tolyl thiourea or di-xylyl thiourea. The increased effectiveness is not merely the sum of the effectiveness of each of the compounds constituting the mixture commonly used, but the composition is superior to either of the ingredients thereof as a flotation promoter. Organic dithiophosphoric acids generally, such as di-alkyl or di-aryl substituted dithiophosphoric acids or their alkali metal salts and the ammonium salts, may be employed in carrying out the present invention. While various dithiophosphates may be utilized in conjunction with di-tolyl thiourea or di-xylyl thiourea, it has been found that excellent results are obtained when certain aryl dithiophosphates, as for example the di-cresyl or the di-xylenyl (mixed) dithiophosphoric acids, are used. As pointed out heretofore these organic dithiophosphoric acid compounds are only capable of dissolving up to about 6% of di-phenyl thiourea, whereas for example di-cresyl dithiophosphoric acid will dissolve as much as 10% of di-tolyl thiourea or di-xylyl thiourea.

This invention will be more fully described in conjunction with the following specific examples. It is to be understood, however, that the examples are for purposes of illustration only and the invention is not to be limited by the details set forth therein.

Tests were carried out on two samples of lead-silver ores. Sample No. 1 was from a mine near Winnemucca, Nevada, and sample No. 2 was from a mine near Silver City, Idaho.

Partial analyses of head samples of the two above ores are shown in Table I.

TABLE I  
PARTIAL ANALYSES OF THE HEAD SAMPLES

| Test procedure              | Ore No. 1 | Ore No. 2 |
|-----------------------------|-----------|-----------|
| Lead..... per cent Pb.....  | 2.71      | 2.12      |
| Silver..... oz. Ag/ton..... | 15.50     | 22.18     |

## GRINDING

A 600-gram sample of minus 20 mesh ore was placed in a laboratory size steel rod mill and diluted with tap water to a pulp density corresponding to 67% solids. Reagents were added as shown in the data of Tables III and IV giving the results of the test work. The ore was then ground for a definite period of time. Screen analyses of the ore pulps obtained during the respective grinding periods employed on each ore are shown in Table II. Ore No. 1 was given a 15-minute grind in all tests, and the ore No. 2 sample was subjected to a 6-minute grinding period in all tests.

was added and the pulp was allowed to condition for 2 minutes. In the balance of the tests, due to the frothing powers of the liquid thiophosphoric acid reagents, it was necessary to add only 0.056 lb./ton cresylic acid to gain sufficient froth volume. At the expiration of 2 minutes conditioning time, the air valve was opened and the resulting concentrate was removed by skimming for a period of 8 minutes. Details of the test procedure and the results obtained will be found in Table III.

## ORE NO. 2

A ground charge of the ore was transferred to a laboratory-size Fagergren flotation machine and diluted with laboratory tap water to approximately 25% solids. The pulp was conditioned for 2 minutes. The air valve was then opened and the resulting concentrate was removed by skimming for a period of 3 minutes. Details of the test procedure and the results obtained will be found in Table IV.

TABLE III  
TESTS ON ORE NO. 1  
Test conditions

| Point of addition | Time, min. | Per cent solids | pH  | Reagents, lbs./ton |                   |                                 |                     |                            |
|-------------------|------------|-----------------|-----|--------------------|-------------------|---------------------------------|---------------------|----------------------------|
|                   |            |                 |     | NaCN               | ZnSO <sub>4</sub> | Na <sub>2</sub> CO <sub>3</sub> | Promoter (variable) | Cresylic acid <sup>1</sup> |
| Grind.....        | 15         | 67              | 8.3 | 0.50               | 1.00              | 15.00                           | 0.115               | 0.112                      |
| Condition.....    | 2          | 22              |     |                    |                   |                                 |                     |                            |
| Flotation.....    | 8          | 22              |     |                    |                   |                                 |                     |                            |

<sup>1</sup> Cresylic acid 0.112 lb./ton used for dry reagents—0.056 lb./ton used for liquid reagents.

## Test results

| Test No. | Promoter (variable) | Feed assay  |             |              | Concentrate |            |                |       | Tailing     |             |      |                |       |
|----------|---------------------|-------------|-------------|--------------|-------------|------------|----------------|-------|-------------|-------------|------|----------------|-------|
|          |                     | Ag, oz./ton | Per cent Pb | Per cent wt. | Assay       |            | Per cent dist. |       | Percent wt. | Assay       |      | Per cent dist. |       |
|          |                     |             |             |              | Ag, oz./ton | Percent Pb | Ag.            | Pb    |             | Ag, oz./ton | Pb   |                |       |
| 1.....   | A.....              | 22.04       | 2.02        | 12.39        | 135.46      | 12.29      | 76.13          | 75.25 | 87.61       | 6.00        | 0.57 | 23.37          | 24.75 |
| 2.....   | B.....              | 21.39       | 1.97        | 8.62         | 178.10      | 15.56      | 71.76          | 68.02 | 91.38       | 6.61        | 0.69 | 28.24          | 31.98 |
| 3.....   | C.....              | 22.08       | 1.95        | 12.94        | 130.22      | 12.19      | 76.31          | 81.03 | 87.06       | 6.01        | 0.43 | 23.69          | 18.97 |
| 4.....   | D.....              | 20.86       | 1.95        | 12.57        | 126.70      | 12.49      | 76.37          | 80.51 | 87.43       | 5.64        | 0.43 | 23.63          | 19.49 |
| 5.....   | E.....              | 21.79       | 2.00        | 14.22        | 119.48      | 11.57      | 77.97          | 82.50 | 85.78       | 5.59        | 0.41 | 22.03          | 17.50 |

A—Thiocarbanilide (alone).

B—Di-o-tolyl thiourea (alone).

C—6% solution of di-phenyl thiourea in di-xylenyl (mixed) dithiophosphoric acid.

D—6% solution of di-o-tolyl thiourea in di-xylenyl (mixed) dithiophosphoric acid.

E—10% solution of di-o-tolyl thiourea in di-xylenyl (mixed) dithiophosphoric acid.

TABLE II  
SCREEN ANALYSES OF GROUND PULPS

| Mesh size  | Per cent weight retained |                        |
|------------|--------------------------|------------------------|
|            | 15 min. grind ore No. 1  | 6 min. grind ore No. 2 |
| +65.....   |                          | 0.55                   |
| +100.....  | 0.63                     | 6.67                   |
| +150.....  | 7.43                     | 17.17                  |
| +200.....  | 91.94                    | 75.61                  |
| Total..... | 100.00                   | 100.00                 |

## FLOTATION

## ORE NO. 1

A ground charge of the ore was transferred to a laboratory-size Fagergren flotation machine and diluted to approximately 22% solids with laboratory tap water. In tests 1 and 2 where thiocarbanilide alone and di-o-tolyl thiourea alone were tested, 0.112 lb./ton of cresylic acid

was added and the pulp was allowed to condition for 2 minutes. In the balance of the tests, due to the frothing powers of the liquid thiophosphoric acid reagents, it was necessary to add only 0.056 lb./ton cresylic acid to gain sufficient froth volume. At the expiration of 2 minutes conditioning time, the air valve was opened and the resulting concentrate was removed by skimming for a period of 8 minutes. Details of the test procedure and the results obtained will be found in Table III.

ORE NO. 2

A ground charge of the ore was transferred to a laboratory-size Fagergren flotation machine and diluted with laboratory tap water to approximately 25% solids. The pulp was conditioned for 2 minutes. The air valve was then opened and the resulting concentrate was removed by skimming for a period of 3 minutes. Details of the test procedure and the results obtained will be found in Table IV.

An analysis of the data of Table III shows that in test 1 when thiocarbanilide alone was used as a promoter the recoveries of silver and lead were better than test No. 2 using di-o-tolyl thiourea alone. The data further shows, however, that the results obtained with the di-tolyl thiourea mixtures were superior to the results obtained with thiocarbanilide alone or di-tolyl thiourea alone, as well as the thiocarbanilide mixtures. Tests Nos. 3 and 4 are comparative and from these it will be seen that the recoveries of silver and lead with the 6% solution of di-tolyl thiourea in di-xylenyl (mixed) dithiophosphoric acid are 76.37 and 80.51% respectively as compared to 76.31 and 81.03% using a 6% solution of di-phenyl thiourea. These results show that the 6% solution of the di-tolyl thiourea is at least the equivalent of a 6% solution of the di-phenyl thiourea; whereas the di-phenyl thiourea alone of test No. 1 is far superior to those of test No. 2 using di-tolyl thiourea alone. In test No. 5 using a 10% solution of di-tolyl thiourea in di-xylenyl (mixed) dithiophosphoric acid, the results are far superior to those of any of the other tests.

TABLE IV  
TESTS ON ORE NO. 2  
*Test conditions*

| Point of addition | Time, min. | Per cent solids | pH  | Reagents, lbs./ton |                   |                                 |                     |
|-------------------|------------|-----------------|-----|--------------------|-------------------|---------------------------------|---------------------|
|                   |            |                 |     | NaCN               | ZnSO <sub>4</sub> | Na <sub>2</sub> CO <sub>3</sub> | Promoter (variable) |
| Grind             | 6          | 67              |     | 0.25               | 1.60              | 1.00                            | 0.115               |
| Condition         | 2          | 25              |     |                    |                   |                                 |                     |
| Flotation         | 3          | 25              | 8.4 |                    |                   |                                 |                     |

*Test results*

| Test No. | Promoter (variable) | Feed assay  |             | Concentrate  |        |       |                | Tailing |              |       |      |
|----------|---------------------|-------------|-------------|--------------|--------|-------|----------------|---------|--------------|-------|------|
|          |                     | Ag, oz./ton | Per cent Pb | Per cent wt. | Assay  |       | Per cent dist. |         | Per cent wt. | Assay |      |
| 1        | F                   | 15.61       | 2.70        | 4.75         | 212.62 | 51.19 | 64.70          | 90.00   | 95.25        | 5.78  | 0.28 |
| 2        | G                   | 15.35       | 2.69        | 5.18         | 196.36 | 46.98 | 66.25          | 90.33   | 94.82        | 5.46  | 0.27 |
| 3        | H                   | 15.32       | 2.65        | 5.94         | 194.64 | 43.18 | 75.46          | 90.60   | 94.06        | 4.00  | 0.10 |

F—6% solution of di-phenyl thiourea in di-xylenyl (mixed) dithiophosphoric acid.

G—6% solution of di-o-tolyl thiourea in di-xylenyl (mixed) dithiophosphoric acid.

H—10% solution of di-o-tolyl thiourea in di-xylenyl (mixed) dithiophosphoric acid.

An analysis of the data of Table IV shows that the recoveries of silver and lead using a 6% solution of di-o-tolyl thiourea in di-xylenyl (mixed) dithiophosphoric acid were 66.25 and 90.33% respectively, as compared to recoveries of 64.70 and 90.00% using a 6% solution of di-phenyl thiourea in di-xylenyl (mixed) dithiophosphoric acid, indicating that the di-tolyl thiourea solution is a more effective promoter than the di-phenyl thiourea solution when used

in equal quantities. The results of test No. 3 show that the use of a 10% solution of di-tolyl thiourea produces results which are greatly superior to the use of the 6% solution of di-phenyl thiourea.

Another series of tests were conducted on ore sample No. 2 and the procedure was essentially the same as that described heretofore. The results of these tests are reported on Table No. V.

TABLE V  
*Test conditions*

| Point of addition | Time min. | Per cent solids | pH  | Reagents, lbs./ton |                   |                                 |                     |               |
|-------------------|-----------|-----------------|-----|--------------------|-------------------|---------------------------------|---------------------|---------------|
|                   |           |                 |     | NaCN               | ZnSO <sub>4</sub> | Na <sub>2</sub> CO <sub>3</sub> | Promoter (variable) | Cresylic acid |
| Grind             | 15        | 67              |     | 0.50               | 1.00              | 15.00                           | 0.115               |               |
| Condition         | 2         | 22              |     |                    |                   |                                 |                     |               |
| Flotation         | 8         | 22              | 8.3 |                    |                   |                                 |                     | 0.056         |

*Test results*

| Test No. | Promoter (variable) | Feed assay  |              | Concentrate  |        |       |                | Tailing |              |       |      |
|----------|---------------------|-------------|--------------|--------------|--------|-------|----------------|---------|--------------|-------|------|
|          |                     | Ag, oz./ton | Pb, per cent | Per cent wt. | Assay  |       | Per cent dist. |         | Per cent wt. | Assay |      |
| 1        | I                   | 22.74       | 2.01         | 12.98        | 126.86 | 12.18 | 72.43          | 78.61   | 87.02        | 7.21  | 0.49 |
| 2        | J                   | 22.72       | 2.02         | 13.87        | 119.00 | 11.51 | 72.67          | 79.21   | 86.13        | 7.21  | 0.49 |
| 3        | K                   | 22.67       | 2.03         | 15.53        | 109.98 | 10.43 | 75.34          | 78.80   | 84.47        | 6.62  | 0.49 |
| 4        | L                   | 22.49       | 2.02         | 16.53        | 105.50 | 9.82  | 77.55          | 80.20   | 83.47        | 6.05  | 0.48 |
| 5        | M                   | 21.97       | 1.99         | 14.18        | 116.84 | 11.15 | 75.42          | 79.40   | 85.82        | 6.29  | 0.48 |

I—6% solution of di-phenyl thiourea in di-xylenyl (mixed) dithiophosphoric acid.

J—6% solution of di-phenyl thiourea in di-xylenyl (mixed) dithiophosphoric acid.

K—10% solution of di-o-tolyl thiourea in di-xylenyl (mixed) dithiophosphoric acid.

L—6% solution of di-(mixed) xylol thiourea in di-xylenyl (mixed) dithiophosphoric acid.

M—10% solution of di-(mixed) xylol thiourea in di-xylenyl (mixed) dithiophosphoric acid.

An analysis of the data in Table V shows that tests Nos. 3, 4, and 5 using solutions of di-tolyl thiourea or di-xylyl thiourea in di-xylényl those of comparative tests Nos. 1 and 2 using solutions of di-phenyl thiourea in di-xylényl (mixed) phosphoric acid.

A series of comparative tests were also conducted on a sample of metallic copper. The results are shown in Table VI.

TABLE VI

| Reagent                                                                              | Feed,<br>per cent<br>Cu | Concen-<br>trate,<br>per cent<br>Cu | Tailing,<br>per cent<br>Cu | Per cent<br>recovery<br>Cu |
|--------------------------------------------------------------------------------------|-------------------------|-------------------------------------|----------------------------|----------------------------|
| 10% solution of di-o-tolyl thiourea in di-xylényl (mixed) dithiophosphoric acid..... | 1.06                    | 16.25                               | 0.40                       | 63.95                      |
| 6% solution of di-phenyl thiourea in di-xylényl (mixed) dithiophosphoric acid.....   | 1.10                    | 11.61                               | 0.69                       | 39.80                      |

The metallurgical results on metallic copper in the above table show that the use of a solution of di-o-tolyl thiourea in di-xylényl (mixed) dithiophosphoric acid improved both the recovery and concentrate grade over the test using a solution of di-phenyl thiourea in di-xylényl (mixed) dithiophosphoric acid.

While in the above description and examples the application of the invention has been described in conjunction with a lead-silver ore, the invention is not limited to these ores as this improved reagent combination is also superior in its results on zinc, copper, gold, as well as other base or other precious metal ores. The substituted di-aryl thioureas may be used in conjunction with other dithiophosphoric acid compounds, as for example, a solution may be made of the substituted di-aryl thiourea with the ammonium salt of di-amyl dithiophosphoric acid. In some cases the mixture of the di-substituted di-aryl thiourea and di-organic dithiophosphoric acid does not remain liquid at ordinary temperatures, and it is usually preferable to add to the solution a suitable diluent such as water, ethyl alcohol, or the like which renders the composition fluid at ordinary temperatures.

It is to be noted that the present invention relates to the use of a reagent combination comprising a solution containing a minor proportion of substituted di-aryl thioureas, such as di-o-tolyl thiourea and di-xylyl (mixed) thiourea and a major proportion of an organic dithiophosphoric acid compound. In the composition of the present invention it is shown that di-tolyl thiourea or di-xylyl thiourea is soluble to the extent of about 10% in di-xylényl (mixed) dithiophosphoric acid and that such a composition is a more effective promoter than similar compositions used heretofore.

From the above it will be apparent that there are numerous possible compositions within the scope of the present invention. Therefore, this invention is to be broadly construed and not to be limited except by the terms of the claims appended hereto.

What I claim is:

1. A composition of matter comprising an or-

ganic dithiophosphoric acid compound and from 6 to 10% of di-tolyl thiourea.

2. A composition of matter comprising an organic dithiophosphoric acid compound and from 5 to 10% of di-xylyl thiourea.

3. A composition of matter comprising di-xylényl dithiophosphoric acid and from 6 to 10% of di-tolyl thiourea.

4. A composition of matter comprising di-xylényl (mixed) dithiophosphoric acid and from 6 to 10% of di-xylyl thiourea.

5. A method of flotation of metal ore values which comprises providing a pulp of ore and water, adding thereto a flotation promoter including a mixture of an organic dithiophosphoric acid compound and from 6 to 10% di-tolyl thiourea, and subjecting the pulp to a froth flotation operation.

6. A method of flotation of metal ore values which comprises providing a pulp of ore and water, adding thereto a flotation promoter including a mixture of an organic dithiophosphoric acid compound and from 6 to 10% di-xylyl thiourea, and subjecting the pulp to a froth flotation operation.

7. A method of flotation of metal ore values which comprises providing a pulp of ore and water, adding thereto a flotation promoter including a mixture of di-xylényl dithiophosphoric acid and from 6 to 10% di-tolyl thiourea, and subjecting the pulp to a froth flotation operation.

8. A method of flotation of metal ore values which comprises providing a pulp of ore and water, adding thereto a flotation promoter including a mixture of di-xylényl (mixed) dithiophosphoric acid and from 6 to 10% di-xylyl thiourea and subjecting the pulp to a froth flotation operation.

9. A composition of matter comprising an organic dithiophosphoric acid having dissolved therein from 6% to 10% of an alkyl substituted diphenyl thiourea.

10. A composition of matter comprising an aryl dithiophosphoric acid having dissolved therein from 6% to 10% of an alkyl substituted diphenyl thiourea.

11. A composition of matter comprising an organic dithiophosphoric acid having dissolved therein from 6% to 10% of ditolyl thiourea, and a diluent.

12. A composition of matter comprising an organic dithiophosphoric acid having dissolved therein from 6% to 10% of di-xylyl thiourea, and a diluent.

13. A froth flotation method for recovery of metal ore values which comprises subjecting an ore containing recoverable metal ore values to a froth flotation treatment in the presence of a promoter comprising an organic dithiophosphoric acid having dissolved therein from 6% to 10% of an alkyl substituted diphenyl thiourea.

14. A froth flotation method for recovery of metal ore values which comprises subjecting an ore containing recoverable metal ore values to a froth flotation treatment in the presence of a promoter comprising an aryl dithiophosphoric acid having dissolved therein from 6% to 10% of an alkyl substituted diphenyl thiourea.

CERTIFICATE OF CORRECTION.

Patent No. 2,330,587.

September 28, 1943.

DAVID WALKER JAYNE, JR.

It is hereby certified that error appears in the printed specification of the above numbered patent requiring correction as follows: Page 4, first column, line 4, before the word "those" insert --(mixed) dithiophosphoric acid are better than--; and that the said Letters Patent should be read with this correction therein that the same may conform to the record of the case in the Patent Office.

Signed and sealed this 16th day of November, A. D. 1943.

(Seal)

Henry Van Arsdale,  
Acting Commissioner of Patents.